

E. H. HINCKLEY,  
PROCESS OF AND APPARATUS FOR PICKLING METALS.  
APPLICATION FILED MAY 20, 1918.

1,434,011.

Patented Oct. 31, 1922.



Inventor.  
Everett H. Hinckley  
by Heard Smith & Tennant.  
Atlys.

Patented Oct. 31, 1922.

1,434,011

# UNITED STATES PATENT OFFICE.

EVERETT H. HINCKLEY, OF NEW BEDFORD, MASSACHUSETTS.

## PROCESS OF AND APPARATUS FOR PICKLING METALS.

Application filed May 20, 1918. Serial No. 235,440.

To all whom it may concern:

Be it known that I, EVERETT H. HINCKLEY, a citizen of the United States, residing at New Bedford, county of Bristol, 5 State of Massachusetts, have invented an Improvement in Processes of and Apparatus for Pickling Metals, of which the following description, in connection with the accompanying drawing, is a specification, like 10 characters on the drawing representing like parts.

This invention relates to a process of and apparatus for pickling or treating metals with acid. While the principles of the invention are of broad application involving the treatment of various metals with various acids the invention is peculiarly valuable in connection with the pickling of iron or steel articles to remove the scale 20 therefrom such as occurs after annealing.

One object of the invention is to minimize the loss of the metal in the pickling operation, the present invention in the case of the pickling of iron or steel articles resulting in a saving of over one-half of the 25 iron lost in the pickling operation in those processes in general commercial use.

Another object of the invention is to effect a saving in the acid employed, the present invention resulting in a large saving in this respect because of the high efficiency 30 of ionization at which the process is carried on.

Another object of the invention is to enable the salt of the metals produced, as for example ferrous sulphate or copperas when iron is pickled with sulphuric acid, to be so concentrated that when the pickling liquor is cooled a large proportion is crystallized and can thus be recovered for commercial purposes without the more tedious and expensive process of evaporation.

Another object of the invention is to enable the supernatant solution at the end of the pickling operation to be of such a character that it may be drawn off and used over again in further pickling operations, the invention enabling this to be done because of the increase in the activity of the solution brought about.

The invention in its main features resides in immersing the metal such as iron in a solution of water and acid such as sulphuric acid of such a degree of concentration and raised to and maintained at such a temperature that maximum efficiency

of ionization and that maximum capacity for absorbing the salt produced as ferrous sulphate which are simultaneously obtainable are thereby secured.

The objects and nature of the invention will appear more fully from the accompanying description and drawings and will be particularly pointed out in the claims.

The single figure of drawing shows more or less diagrammatically a simple and preferred form of apparatus embodying the invention and by the use of which the process embodying the invention may be practiced.

The process and apparatus are particularly useful in connection with the pickling of iron or steel articles such for example as the comparatively thin plates from which nails or tacks are produced and for convenience of disclosing the invention will be described in connection therewith, but it is to be understood that it is equally applicable to the treatment of other metals with other acids.

The invention is based upon securing and correlating a proper degree of concentration in the acid solution and a temperature of that solution during the pickling operation which will secure the most efficient or most active ionization of the acid which can be obtained simultaneously with the greatest capacity of this solution for absorbing the salt produced; in other words, the idea of this invention is to secure that maximum efficiency of operation and that maximum capacity of product which it is possible to secure simultaneously. It will be obvious also that the invention may be substantially secured without reaching this maximum of perfection and a reasonable variation in either direction is considered as coming within the scope of the invention.

The efficiency of the ionization of the acid solution increases as the concentration of the solution decreases. Sulphuric acid, for example, at its strong commercial strength of about 96% is so filled with molecular  $H_2SO_4$  that practically no ionization can take place. Under the practice now commonly prevailing a solution of about 15% is commonly employed which at a temperature of about 20° C. permits of approximately 23% of ionization or in other words approximately 23% of the  $H_2SO_4$  molecules in the solution are in the form of ions. This percentage of ionization in-

creases as the percentage of concentration of the solution decreases so that with a solution of one-half of one percent of sulphuric acid it is found that there is about 5 60% of ionization.

The increase of the temperature of the solution also acts to increase the ionization in proportion to the increase in the volume caused thereby and in proportion to the increased heat content of the ions. 10

While the efficiency of ionization thus rapidly increases as the concentration of the solution decreases it will be seen that the capacity of the operation is reduced. For 15 example, if the solution should be so decreased in concentration as to result in complete ionization of the acid the capacity of the operation would be very slight and the product of the pickling operation would be 20 practically nothing but all acid present would be utilized.

The capacity of the operation is determined by the amount of the salt produced, in this case ferrous sulphate  $\text{FeSO}_4$ , which 25 can be absorbed by or go into solution in the solution.

It has been found that for practically any degree of concentration of the solution a temperature of  $90^\circ \text{ C}$ . produces a condition 30 in which  $\text{FeSO}_4$  has its maximum solubility and the temperature at which other salts have their maximum solubility and other acids their most efficient ionization may readily be determined by experiment.

The increase of temperature of the solution also acts to decrease the solubility of the solution for hydrogen gas and as hydrogen gas results from the union of the hydrogen ions produced in ionization and is 40 freed it follows that the raising of the temperature in this way also enables the production of further  $\text{FeSO}_4$  and thus increases the efficiency and capacity of the operation.

There is therefore a point at which a certain concentration of the solution raised to 45 and maintained at a certain temperature will produce the maximum ionization and the maximum amount of salt, that is, the point at which the greatest efficiency and greatest capacity that can be simultaneously obtained are in fact obtained.

In the case of the pickling of iron with sulphuric acid this is found to be when the sulphuric acid solution is at substantially 55 one-half percent concentration and when the temperature is at substantially  $90^\circ \text{ C}$ . Any substantial variation either in the degree of concentration or in the temperature either reduces both the efficiency and capacity of 60 the operation or increases the one at the expense of the other with a total loss in each case.

This process it will be seen prevents any danger of the crystallization of the salt upon 65 the article to be pickled because the solu-

tion can never reach such a degree of concentration that the salt will be produced more rapidly than it can be dissolved by the solution. This condition has frequently obtained in commercial processes in practice 70 and results in a super-saturated solution being formed locally around the article and a consequent crystallization of the salt upon the article which insulates it from the action of the acid and destroys or materially hinders the pickling operation. This process also by maintaining an even and constant action of the solution, prevents the solution from becoming "dead" as frequently happens in present commercial practice due 75 to the oxidization of the ferrous to the ferric ion.

In the drawings there is illustrated a simple and preferred form of apparatus by which the process of this invention may be 80 carried on. As shown the articles to be pickled are iron plates 1 such as employed in the manufacture of tacks and nails. These plates are suitably supported on edge and held separated from each other by a 85 suitable skeleton frame 2 which by means of supporting chains 3 may be handled from a crane or derrick. The frame 2 is made of bronze or other material not subject to the action of the pickling solution. 90

A vat 4 of a size suitable to receive and cover the frame 2 with its supported plates 1 is provided. This vat is provided with means by which it may be filled with water and with means by which an amount of 100 acid may be automatically supplied thereto to give the required concentration of solution in quantities sufficient to pickle the quantity of plates or articles carried by the frame. 105

The amount of acid supplied to the solution may be automatically determined by a variety of means one form of which is herein illustrated as a tank 5 to which a pipe 6 leads from a suitable source of acid 110 supply. The flow from the pipe 6 is controlled by a valve 7 operated by a float 8. The tank 5 discharges into the vat 4 through the pipe 9 the upper end of which is provided with a siphon valve 10 raised by a connection 11 to a trip lever 12 located in the descending path of the frame 2. This is so arranged that as the frame 2 is lowered into the vat 4 it strikes the trip lever 12 and as a result discharges the contents of the tank 115 5 into the vat 4. This general type of means for discharging a predetermined quantity of liquid from the tank 5 into the vat 4 is shown in the patent to Craigie No. 433,447 granted August 5, 1890. It will thus be seen that by a simple calculation based upon the surface area of the articles 1 to be pickled, the contents of the tank 5 discharged upon the raising of the siphon valve 10, the strength of the acid in the tank 5, 120

130

and the quantity of water in the vat 4, that the degree of concentration of the solution produced in the vat 4 may be automatically and accurately secured.

5 The desired temperature of the solution in the vat 4 may be obtained in any suitable manner and for that purpose a steam pipe 13 connected to a suitable source of steam supply 14 extends into the vat 4 and opens 10 near the bottom thereof. A thermostatically controlled valve 15 is provided in the pipe 13. This valve is of a familiar type operated by a thermostat 16 containing an expansible liquid which in turn operates 15 through a flexible connection 17 the movable parts of the valve 15. When this thermostat is set to operate at a desired temperature as, for example, 90° C., it will automatically act by the opening and closing 20 of the valve 15 to supply the steam necessary to raise the solution to and maintain it at the desired temperature. It is found that the condensate from the steam pipe will in practice about equal the evaporation so 25 that this means of maintaining the temperature has no appreciable effect upon the degree of concentration of the solution.

At the conclusion of the pickling operation practiced in accordance with this invention the resultant solution will be found 30 to be of such a high degree of concentration that when it is cooled a large proportion of the salt produced such as ferrous sulphate will crystallize and may be recovered for 35 commercial purposes simply by drawing off the supernatant liquor. This is a very valuable feature of the process because heretofore the general practice has been to secure the salt by evaporation which requires time 40 and is expensive. A further valuable feature is due to the fact that the salt crystallizes spontaneously and gradually and is therefore recovered in a more chemically pure state.

45 Furthermore, the supernatant liquor itself is a solution of sulphuric acid and water and uncrystallized ferrous sulphate and is not only of sufficient strength but in fact of greater strength than is necessary for use in 50 continuing the future pickling operations. This is due to the decreased concentration of the  $\text{SO}_4$  ion; that is to say, in this solution the  $\text{SO}_4$  ion exists in small numbers so as not to oppose the decomposition of 55 molecular sulphuric acid into its ions.

The supernatant liquor is therefore drawn off into another vat and by the addition of the proper amounts of water and fresh sulphuric acid brought to the desired degree 60 of concentration. This may be done in various ways.

In the drawings a second vat 18 is located adjacent the vat 4 and connected thereto by a pipe 19 provided with valves 20 and 21. 65 Between these valves a pipe 22 is connected

to the pipe 19 and extends to a steam injector 23 connected to the source of steam supply 14. At the conclusion of the pickling operation in the vat 4 and after the solution therein has cooled the valve 20 is 70 opened, the valve 21 being closed, and steam is turned on by the valve 24 thus injecting the supernatant liquor in the vat 4 into the vat 18.

Then the required amount of water and 75 acid from a second tank 25 is introduced into the vat 18 to bring the solution up to the required degree of concentration as one-half of one percent. The valve 24 is then closed and the pipe 13 swung over into the 80 vat 18 and the thermostat 16 placed in the vat 18 whereupon the vat 18 is ready for a second pickling operation.

At the conclusion of this pickling operation the injector 23 is swung over into the 85 vat 4 and the supernatant liquor drawn from the vat 18 into the vat 4 in a manner similar to that just described. Thus by means of an apparatus such as that disclosed the pickling operation may be carried on indefinitely.

The process of applying the solution to the metal has been referred to herein as that of "immersion" but it is to be understood that this term is to be taken as including 95 any process by which the solution is applied so as to cover the surface of the metal to be acted upon.

Having fully described my invention, what I claim as new and desire to secure by 100 Letters Patent is:

1. The process of pickling iron which consists in immersing the iron in a solution of water and sulphuric acid of such a degree of concentration and raised to and maintained at such a temperature that that maximum efficiency of ionization and that maximum capacity for absorbing ferrous sulphate which are simultaneously obtainable are thereby secured. 110

2. The process of pickling iron which consists in immersing the iron in a solution of water and substantially one-half of one percent of sulphuric acid and raising the solution to and maintaining it at substantially 115 90° C. whereby substantially that maximum degree of efficiency of ionization and substantially that maximum capacity for absorbing ferrous sulphate which are simultaneously obtainable are thereby secured. 120

3. In the process of pickling iron in a solution of water and sulphuric acid the step which consists in maintaining said solution at a temperature of approximately 90° C.

4. The process of pickling metal which 125 consists in immersing the metal in a solution of water and acid and in maintaining the concentration of the solution at or below that point at which all the salt produced will be dissolved by the solution. 130

5. The process of pickling metal which consists in immersing the metal in a solution of water and acid and in maintaining the solution at such a temperature and at such a 45  
 5 degree of concentration that the maximum number of hydrogen ions which can be economically utilized are formed in the solution.
6. The process of pickling metal defined in claim 1 together with the additional steps 50  
 10 of allowing the solution to cool at the end of the pickling operation, removing the supernatant liquid, adding thereto amounts of water and acid dependent upon the surface area of a second batch of metal to be  
 15 pickled sufficient to give the required concentration of solution, immersing the second batch in the solution and maintaining the solution at such a temperature that that maximum efficiency of ionization and that maximum capacity for absorbing the salt produced which are simultaneously obtainable are thereby secured.
7. The process of pickling metal defined in claim 1 which consists in addition in allowing the solution to cool and thus permitting the salt produced to crystallize spontaneously and gradually thus producing a substantially chemically pure salt, and in removing the supernatant liquor. 60  
 25
8. An apparatus for pickling metal which consists in a vat adapted to contain the pickling solution, means for automatically supplying an amount of acid to said vat sufficient to give a predetermined degree of concentration to the solution, and means for automatically maintaining the temperature of the solution at a predetermined point during the pickling operation. 65  
 30
9. An apparatus for pickling metal which consists in a vat adapted to contain a pickling solution, means for automatically supplying an amount of acid to said vat suffi- 70  
 40

cient to give a predetermined degree of concentration to the solution, means for supplying steam to said solution, a valve in said steam supply, a thermostat in said solution operatively connected to said valve and acting automatically to supply sufficient steam to maintain said solution at a predetermined degree of temperature. 75  
 50

10. An apparatus for pickling metal as defined in claim 8 comprising in addition a second vat and means for drawing off the supernatant liquor from the solution in the first vat when cooled and discharging it into the second vat. 55

11. The process of pickling metal which consists in immersing the metal in a solution of water and acid having a degree of concentration within such a range and raised to 60 and maintained at a temperature within such a range that substantially the same proportion of salt will be crystallized out for any degree of concentration within said range provided the temperature within its 65 range be inversely proportioned.

12. The process of pickling iron which consists in immersing iron in a solution of water and sulphuric acid having the concentration ranging from one half of one percent to ten percent of sulphuric acid and raising the solution to and maintaining it at a temperature ranging from ninety degrees C. to seventy-five degrees C. according to the concentration whereby substantially 70 the same proportion of ferrous sulphate will be crystallized out whatever be the degree of concentration within the range stated provided the temperature is inversely proportioned thereto within the range stated. 75  
 80

In testimony whereof, I have signed my name to this specification.

EVERETT H. HINCKLEY.